

# UNITED STATES PATENT OFFICE.

TOMOTAKE HONDA, OF ONGAGUN, JAPAN, ASSIGNOR TO HEIJIRO NISHIMURA, OF TOKYO, JAPAN.

## PROCESS FOR MANUFACTURING OF AN ELASTIC IMITATION HEMP.

1,351,385.

Specification of Letters Patent. Patented Aug. 31, 1920.

No Drawing.

Application filed July 3, 1919. Serial No. 308,368.

To all whom it may concern:

Be it known that I, TOMOTAKE HONDA, subject of the Empire of Japan, residing at No. 1530, Orio, Ongagun, Fukuoka, Japan, have invented certain new and useful Improvements in Processes for Manufacturing of an Elastic Imitation Hemp, of which the following is a specification.

This invention relates to process for the manufacturing of an elastic imitation hemp by treating cotton thread or cotton cloth, and it consists in coating the material with a size or paste made from the roots of the hydrosme rivieri and then subjecting the coated cotton thread or cotton cloth to tannic acid, and if desired to a further treatment of sodium stannate or sodium silicate.

The object of this invention is to give a hemp-like appearance and high elasticity to the cotton thread or cotton cloth and also to give high resistance for washing, rubbing and sweat, that is to say, is to obtain an imitation hemp cheaply.

If a solution of tannic acid is added to a solution of size or paste made from the roots of the hydrosme rivieri the paste so formed is converted instantly into a white insoluble substance. The reaction is very complete and no trace of the paste remains in the solution. This white precipitate is a special compound to be called "tannin hydrosme rivieri" and has a high elasticity and is not affected appreciably by acids or other alkalis excepting sodium stannate or sodium silicate, by action of which the precipitate is rendered translucent.

The above mentioned reaction is the origin of this invention.

To practice this invention, the refined cotton thread is drawn passing firstly through a solution of hydrosme rivieri size, (if some weight is wanted, a suitable quantity of metal salts, such as tin, antimony, aluminum or chromium may be added to the konnyaku-nori) and nextly through a 0.5-1.00 % solution of tannic acid and then wound on a reel.

After the material has been wound upon the reel, it is removed from the same in a wet condition, dried, when the insoluble tannin hydrosme rivieri is found among the fiber. (If metal salt is added, the tannin metal salt is contained in the tannin hydrosme rivieri). When dried it is washed with water and dried again.

By these treatments the nap on the material is laid down and in appearance resembles hemp very nearly.

If translucence is wanted, the thread, treated as above mentioned, is to be boiled about 5 minutes in a 0.3-0.7 % solution of sodium stannate or in a 1-3 % solution of sodium silicate, then it becomes translucent and has a luster for the reason that the tannin hydrosme rivieri itself became translucent.

In the manufacturing of imitation hemp heretofore, the cotton thread was passed through a size, and wound firstly on a small reel to be dried. In winding on small reel, the size was pressed out on the surface, hence the thread was coated unevenly by the size. When dried on the small reel, the thread must be wound again on a larger reel. During this re-reeling a great deal of nap is formed on the thread for the reason that the thread on the small reel adheres.

In this application, however as the hydrosme rivieri size loses its adhesion instantly by the action of the tannic acid, the thread may be wound directly on the larger reel, without the necessity of drying on the small reel. The nap may be laid down by the tannin hydrosme rivieri and it will never nap as there is no adhesion between the threads.

The tannin hydrosme rivieri has a mordanting property for the basic dyestuff, consequently no mordant is needed in dyeing the thread with the basic dyestuff.

Having now particularly described and ascertained the nature of my said invention and in what manner the same is to be performed, I declare that what I claim is:

1. The process for manufacturing elastic imitation hemp from cotton thread or cloth, consisting of first coating the cotton thread or cloth with a size or paste made from the roots of the hydrosme rivieri and then treating the same with tannic acid.

2. The process for manufacturing elastic imitation hemp from cotton thread or cloth, said process consisting of first coating cotton thread or cloth with a paste or size made from the roots of the hydrosme rivieri, then treating the same with tannic acid and finally treating the same with sodium stannate.

3. The process for manufacturing elastic imitation hemp from cotton thread or cloth,

said process consisting of first coating cotton  
thread or cloth with a paste or size made  
from the roots of the hydrosme rivieri, then  
treating the same with tannic acid, and  
5 finally treating the same with a substance  
which will render it translucent.

In testimony whereof I have hereunto set

my hand in presence of two subscribing wit-  
nesses.

**TOMOTAKE HONDA.**

Witnesses:

TSUNEZO SHIGO,  
S. SASADA.